

Patented Mar. 30, 1926.

1,578,896

# UNITED STATES PATENT OFFICE.

GUY LEONARD, OF BALTIMORE, MARYLAND.

## STENCIL SHEET.

No Drawing.

Application filed December 17, 1925. Serial No. 76,105.

To all whom it may concern:

Be it known that I, GUY LEONARD, a subject of the King of Great Britain, residing in Baltimore, in the county of Baltimore and State of Maryland, have invented certain new and useful Improvements in Stencil Sheets, of which the following is a specification.

This invention relates to stencil-sheets for typewriting and other work, and its principal object is to produce an inexpensive, pliable, strong, durable and efficient stencil-sheet economical of ink, which can be stencilled in dry condition, and is not injured by rough handling, and will yield a large number of copies.

A sheet of Yoshino or other loose-fibred paper is coated by liquid which includes a large proportion of shellac solution in methyl alcohol or other solvent. With the shellac solution there is employed a solution of aluminum stearate (a salt of stearic acid) in benzol, partly for imparting a water-proof quality to the sheet, but mainly for combining thoroughly with the shellac and making more of a film. The aluminum stearate overcomes the brittleness of the dry shellac, so that instead of the film being likely to be shattered by the type, it is rendered tough and elastic, and is sharp-cutting. The aluminum stearate conduces to durability of the sheet, which yields many more copies than would be possible with a sheet having only a shellac film. The aluminum stearate combines thoroughly with the shellac, and makes more of a film on the sheet, and makes the film more elastic.

To the solution of aluminum stearate in benzol, to which is added a solution of shellac in methyl alcohol, there is also added the following in a butyl alcohol solution, namely diethylphthalate, triacetin, acetanilid and triphenolphosphate. The butyl alcohol forms a solvent for said substances.

Among other suitable solutions for the aluminum stearate are amylacetate and gasoline. Among other solutions for the shellac are methyl acetone, acetone, amylacetate and denatured alcohol. The aluminum stearate may be dissolved in amylacetate or gasoline.

The aforesaid preparation is heated to about 70 degrees centigrade and is then cooled to about 50 degrees centigrade. Then there is thoroughly mixed therewith a mix-

ture of castor oil, oleic acid and neat's-foot oil. The resulting preparation is then applied to the paper.

For the stearate - benzol - shellac - alcohol preparation, there are preferably used 40 parts aluminum stearate, 80 parts benzol and 200 parts shellac solution in methyl alcohol 40 per cent.

For the butyl alcohol solution, there may be employed the following: 80 parts butyl alcohol, 50 parts triacetin, 80 parts diethylphthalate, 10 parts acetanilid, and 10 parts triphenolphosphate.

The oil mixture is preferably 80 parts castor oil, 20 parts oleic acid and 20 parts neat's-foot oil.

All of the above proportions are by weight. The proportion given for each ingredient holds good for the entire coating solution, as, for example, the neat's-foot oil may be equal to  $\frac{1}{10}$  by weight of the shellac solution.

Triacetin is a glycerol fatty acid ester. By the aid of the triacetin, it is designed to improve the pliability and elasticity in the stencil-sheet; the triacetin being a plastifier. Since alcohol evaporates from the coated sheet, the weight of the various other ingredients may finally be somewhat different from that given in the foregoing formula. Triacetin and oil are mutually soluble in alcohol or ether or acetone, or any of the common solvents for shellac. The diethylphthalate is an added softening or tempering ingredient, which is also soluble in alcohol or the other common solvents, thus making with the shellac, triacetin, etc., a homogeneous dry coating upon the evaporation of the solvent.

The proportions may be varied within the scope of the invention, and there is permissible some latitude of variation in the ingredients themselves, as, for example, glycerin may be used as a substitute softening agent; or the softening agents may be modified by glycerin or other ingredient.

The coating preparation can be colored with any dye that is soluble in alcohol, or in a common solvent of the solution.

The coating solution may be prepared preferably by first dissolving the aluminum stearate in benzol, then adding the shellac solution, then mixing the liquid triacetin, diethylphthalate, acetanilid, and triphenol-

phosphate in a butyl alcohol solution, and adding this mixture to the foregoing. This preparation may then be heated to about 70 degrees centigrade, and then cooled to about 50 degrees centigrade. This heat will be usually sufficient for the oil ingredients. Then the mixture of castor oil, oleic acid and neat's-foot oil is thoroughly admixed with said preparation. In this bath the 10 Yoshino paper sheets may be immersed, or the sheets may be floated upon the liquid. Excess of liquid may be removed from the sheet, and the same may be hung up to dry, whereupon it is ready for use in the type-writing machine.

The invention is not limited to the proportions given, nor to the exact ingredients named, and variations may be resorted to in carrying out the process. It is not necessary in all cases to employ the entire formula, as portions thereof may be used within the scope of the invention.

I claim:

1. A stencil-sheet of loose-fibred paper 25 coated with a solution of shellac, aluminum stearate, diethylphthalate, triacetin, acetanilid, triphenolphosphate, castor oil, oleic acid and neat's-foot oil.
2. A coating bath for a stencil-sheet of 30 loose-fibred paper having substantially the following ingredients and proportions thereof by weight, viz: aluminum stearate 40 parts; benzol 80 parts; shellac solution in methyl alcohol 40 per cent., 200 parts; triacetin 50 parts; diethylphthalate 80 parts; acetanilid 10 parts; triphenolphosphate 10 parts; butyl alcohol 80 parts; castor oil 80 parts; oleic acid 20 parts; and neat's-foot oil 20 parts.
3. The process of dissolving aluminum 40 stearate in benzol, adding a solution of shellac in methyl alcohol, mixing therewith a butyl alcoholic solution of diethylphthalate, triacetin, acetanilid and triphenolphosphate, and incorporating with the aforesaid preparation a mixture of castor oil, oleic acid and neat's-foot oil.
4. The process of dissolving aluminum 50 stearate in benzol, adding a solution of shellac in methyl alcohol, mixing therewith a butyl alcoholic solution of diethylphthalate, triacetin, acetanilid and triphenolphosphate; heating the aforesaid preparation to about 70 degrees centigrade, cooling the same to about 50 degrees centigrade, and incorporating therewith a mixture of castor oil, oleic acid and neat's-foot oil.
5. A stencil-sheet of loose-fibred paper 55 coated with shellac tempered by aluminum

stearate and softened by oil or fatty material.

6. A stencil-sheet of loose-fibred paper 60 coated with shellac tempered by aluminum stearate and triacetin, and softened by an oily or fatty preparation.

7. A stencil-sheet of loose-fibred paper 65 coated with shellac tempered by aluminum stearate, triacetin and diethylphthalate, and softened by an oily or fatty ingredient.

8. A stencil-sheet of loose-fibred paper 70 coated with shellac tempered by aluminum stearate, triacetin and diethylphthalate, and acetanilid to which is added a suitable softening or shortening ingredient.

9. A stencil-sheet of loose-fibred paper 75 coated with shellac tempered by aluminum stearate, triacetin and diethylphthalate, acetanilid and triphenolphosphate incorporated with a softening or shortening agent.

10. A stencil-sheet of loose-fibred paper 80 coated with shellac tempered by aluminum stearate and triacetin, and softened by a mixture of castor oil, oleic acid and neat's-foot oil.

11. A stencil-sheet of loose-fibred paper 85 coated with shellac tempered by aluminum stearate, triacetin, diethylphthalate and acetanilid, and softened or shortened by castor oil, oleic acid and neat's-foot oil.

12. A stencil-sheet of loose-fibred paper 90 coated with shellac tempered by aluminum stearate, triacetin, diethylphthalate and acetanilid incorporated with castor oil, oleic acid and neat's-foot oil.

13. An ink-proof coating bath for paper, 95 having about 320 parts by weight of a shellac solution in alcohol and aluminum stearate solution in benzol, about 230 parts by weight of a butyl alcohol solution of triacetin, diethylphthalate, acetanilid and triphenolphosphate, and about 120 parts by weight of a preparation of castor oil, oleic acid and neat's-foot oil.

14. The process of dissolving aluminum 100 stearate in benzol, adding a solution of shellac in methyl alcohol, mixing therewith a butyl alcoholic solution of diethylphthalate, triacetin, acetanilid and triphenolphosphate, heating the aforesaid preparation to about 70 degrees centigrade, cooling the same to 110 about 50 degrees centigrade, incorporating therewith a mixture of castor oil, oleic acid and neat's-foot oil, coating a loose-fibred paper with the aforesaid coating, removing surplus coating from the paper, and drying 115 the paper.

GUY LEONARD,